

Feb. 19, 1963

A. BROWN ET AL

3,078,139

PROCESS FOR PRODUCING POLYSTYRENE FIBERS

Filed Oct. 31, 1958

2 Sheets-Sheet 1



INVENTORS  
ALEXANDER BROWN  
CHARLES N. MERRIAM  
WALTER A. MILLER

BY *Walter C. Kehm*  
ATTORNEY

Feb. 19, 1963

A. BROWN ET AL

3,078,139

## PROCESS FOR PRODUCING POLYSTYRENE FIBERS

Filed Oct. 31, 1958

2 Sheets-Sheet 2

Fig. 2.



INVENTORS  
*ALEXANDER BROWN  
CHARLES N. MERRIAM  
WALTER A. MILLER*

BY *Walter C. Kehm*  
ATTORNEY

## 1

3,078,139

PROCESS FOR PRODUCING POLY-  
STYRENE FIBERS

Alexander Brown, Basking Ridge, Charles N. Merriam, Florham Park, and Walter A. Miller, Somerville, N.J., assignors to Union Carbide Corporation, a corporation of New York

Filed Oct. 31, 1958, Ser. No. 771,023

5 Claims. (Cl. 18—54)

This invention relates in general to the production of synthetic fibers and monofilaments. More particularly, it relates to novel fibers and monofilaments formed from isotactic polystyrene and to a novel melt spinning process for producing these fibers and monofilaments.

Heretofore, monofilaments and particularly fibers formed from conventional, i.e., sterically random polystyrene have generally been unsuited for many commercial uses because of their extremely poor solvent resistance and poor dimensional stability at elevated temperatures. Especially has this been found to be true in applications relating to the textile art.

Recent developments, however, have led to the development of methods for producing isotactic polystyrene, i.e., styrene homopolymer chains which are sterically regular along substantially the entire chain length or at least along a considerable portion thereof. Isotactic polystyrene, because of its inherent ability to crystallize, offers several outstanding properties desirable in fibers or filaments for textile uses, such as high strength, high stiffness, and unusual chemical resistance. The isotactic polymer is useful for textile purposes only if methods are found to process the polymer raw material so that the products possess and/or maintain these useful properties, and at the same time overcome the problems incurred by the extremely low impact strength or brittleness which characterizes the isotactic polymer.

The method for forming fibers from conventional polymers generally referred to as melt spinning has heretofore not been adaptable to forming textile quality fibers of isotactic polystyrene. One of the major reasons has been the inability to molecularly orient the polymer molecules in the fibers uniformly and to a degree sufficient to obtain the strength, dimensional stability, and flexibility required. Although other methods have been proposed for forming isotactic polystyrene fibers, those methods are for the most part complicated, expensive, or fail to produce textile quality fibers.

It is therefore the general object of the present invention to provide a process for producing superior crystalline isotactic polystyrene fibers by the method of melt extrusion or melt spinning.

This general object and other more particular objects which will be apparent from the specification are accomplished in accordance with the present invention by the method which includes the steps of melt extruding an isotactic polystyrene having a melt index of between 1 and 20 through a fiber forming die at a temperature between about 230° C. and 330° C., hot drawing the fibers as they emerge from the forming die while maintaining the fibers at substantially the extrusion temperature, and thereafter cold drawing the fiber to impart a degree of stretch of from about 800 to 900 percent whereby a high degree of molecular orientation is induced in said fiber.

Several methods for polymerizing styrene to form the isotactic form of polystyrene have recently been proposed. More specifically, one such method is described in detail in pending United States application Serial No. 577,190, filed April 10, 1956, now abandoned. In general, the isotactic polymer obtained directly from the polymerization autoclave has such an exceedingly high melt viscosity, i.e., very low melt index, that melt spinning of the un-

## 2

treated polymer to produce fibers of any quality is not possible.

Therefore, in carrying out the process of the present invention, virgin isotactic polystyrene having a melt index of about .01 (250° C., 44 p.s.i.) as initially produced is subjected to controlled pyrolysis or thermal cracking to increase the melt index to about 10 and preferably not greater than about 20. The pyrolyzed polymer is then extruded and metered through the orifices of a spinneret and passed through a heated zone maintained at a temperature substantially the same as the spinneret die whereby any molecular orientation resulting from the shearing stresses exerted on the polymer as it passes through the small orifices of the spinneret is removed. Following this 10 high temperature relaxation step the fibers are stretch oriented under conditions which permit the polymer to become crystalline. As used throughout the specification, examples and claims, the melt index values were determined on an I.C.I. grader at 250° C. with a ram pressure of 44 p.s.i. according to ASTM test method 1238—52T.

Pyrolysis of the isotactic polystyrene prior to the melt spinning operation may be accomplished by several methods with comparable results. While the method employed is by no means critical insofar as the overall process of the present invention is concerned, it has been found, however, that increasing the melt index of an isotactic polystyrene polymer by pyrolysis imparts beneficial properties to the fibers produced therefrom which are not evident when an isotactic polystyrene having the same melt index as the pyrolyzed polymer is prepared directly by polymerizing monomeric styrene. It is therefore preferred that the material processed according to this invention be initially pyrolyzed.

Illustratively, in one preferred method the isotactic polystyrene is fed to a one and one-quarter inch Hartig extruder fitted with a single flight metering screw and having a barrel diameter of 1 and 1/4 inch (manufactured by the Hartig Engine and Machine Company, Inc., Hillside, New Jersey). The barrel of this extruder is maintained at a temperature between 250° C. and 300° C. The head of the extruder is fitted with a heating chamber, referred to hereinafter as the "heated tube." The heated tube is a straight one inch bore stainless steel or Hastelloy tube which is approximately 12 inches long and is fitted with an internal torpedo consisting of a stainless steel rod running longitudinally in the tube. The torpedo is of such a cross-sectional diameter as to form an annular space between itself and the inner wall of the tube, said 35 annular channel being from about 1/32 to about 1/16 of an inch in thickness. As the isotactic polystyrene is forced through this annular channel under the pressure exerted by the extruder, it is heated by electrical heaters banding the outside of the tube. The temperature of the tube and 40 the molten polystyrene in the annular channel is measured by appropriately located thermocouples. The residence time for the polystyrene in the heated tube and the temperature at which it is treated depend for the most part upon the initial melt index of the polymer and the desired 45 melt index of the pyrolyzed product. In general, however, maintaining a constant temperature in the range of 350° C. to 425° C. uniformly throughout the polymer in the heated tube for a period of about 90 seconds is sufficient to pyrolyze a polymer having an initial melt index of 50 about .01 at 250° C. to a polymer having a melt index of about 10 at 250° C. Advantageously the modified polystyrene flowing from the heated tube is passed directly into a rotating disc viscosimeter operating in a pre-determined temperature range. This instrument continuously indicates the product melt viscosity, which in turn 55 is used to control the temperature of the heated tube so that a constant melt viscosity of the product is assured.

From here the product is extruded as a rod, and fed to the extruder provided with the spinneret die, or is passed through a quenching bath, and then to a dicer for pelletizing.

In a second method, the isotactic polystyrene is treated in a "heated mill" which continuously mills and heat treats the polymer. The essential feature in such a mill is the use of helically-threaded rolls which are rotated in opposite directions to draw the polystyrene into the bite of the rolls. These rolls are housed in such a manner that a heating jacket is provided and there is a chamber over at least part of the threaded portion of the roll whereby the material can be heat treated in the presence of an inert gas such as nitrogen or subjected to a vacuum during the thermal treatment. Under these operating conditions the polymer is repeatedly worked as it passes through the bite, blended to assure temperature uniformity, and conveyed along the rolls to the discharge end by the helical threads. Generally the polystyrene is preheated to about 300° C. before it enters the mill which is heated by passing hot liquids or vapors through the heating jacket. The ultimate temperature attained by the polystyrene, the period of time during which this temperature is maintained, and the initial melt viscosity of the polystyrene are interdependent factors which may be determined by routine experimentation to obtain the final pyrolyzed polystyrene product having the desired increased melt index.

The melt viscosity of the pyrolyzed isotactic polystyrene which is melt spun into fibers depends to a large extent upon the diameter of the orifices in the spinneret die since the polymer must be capable of being forced through the die orifices at a temperature which does not bring about any substantial degradation of the polymer. While the melt index range of the polystyrene found suitable for melt spinning according to the present process is therefore by no means critical, it has been found however that a melt index range of from about 1 to about 30 is generally suitable, with the preferred range being about 2 to about 20 at 250° C. (ASTM 1238-52T).

Although isotactic polystyrene polymers having melt indices over a rather wide range may be melt spun, the temperature range for extrusion of these polymers through the die of the spinneret is quite narrow. The minimum extrusion temperature is, of course, at least as high as the first order transition temperature, and is as much higher than the first order transition temperature as practical considerations of the pressure required to force the material through the die orifices permit. Irrespective of the melt index within the limits set forth above, i.e., about 1 to about 20 at 250° C., the minimum extrusion temperature for the purposes of this invention is at least 230° C. An extrusion temperature of about 250° C. to about 300° C. is particularly preferred.

The maximum extrusion temperature has as the sole limiting factor, in the case of isotactic polystyrene, thermal degradation of the polymer. At temperatures above about 330° C. molecular degradation of the material in the spinneret is sufficient to seriously impair the physical properties of the spun fibers. For this reason the generally preferred extrusion temperature range is at least 230° C. and not more than about 330° C.

The isotactic polystyrene filaments as they are formed by the passing of the molten polymer mass through the spinneret die orifices are subjected to shearing stresses which induce a substantial degree of molecular orientation. Within the narrow range of temperatures found suitable for extrusion, the shear induced molecular orientation at the surface of the filament is not permitted to relax when the filament emerges from the spinneret into ambient room temperature because the chilling effect of room temperature air is sufficient to cool the surface of the fiber to a point where relaxation is not possible. The internal portion of the filament, however, because of the relatively poor heat conductivity of the polystyrene, is

sufficiently warm to permit relaxation of the stress induced orientation. Further, since the extruded filaments must be reduced in diameter for most textile uses by drawing down as they leave the spinneret, additional orientation would occur in the cooled outer portions of the filaments. Therefore when filaments having a partially oriented surface and an unoriented interior are subjected to "cold stretching" for the purpose of inducing controlled uniform molecular orientation to increase the strength of the filaments, the molecules at the surface orient to their fullest extent before full orientation of the internal molecules occurs. As a result, such filaments can never be fully and uniformly oriented to the extent that they possess the requisite fiber strength, toughness, and crystallinity to ensure dimensional stability at elevated temperatures.

For this reason, in the process of this invention the isotactic polystyrene filaments are not chilled or permitted to become chilled as they leave the spinneret and are subjected to draw-down to bring about a size reduction. This is contrary to prior known melt spinning procedures involving other plastic materials including non-isotactic polystyrene in which a jet of cold air is conventionally directed across the filament at the point where it emerges from the forming die. Instead, we have discovered that it is vital that provision be made for maintaining the temperature of the filaments uniformly at the die temperature during the period of size reduction draw-down for a period of time sufficient to allow any oriented molecules at the surface of the filaments to relax whereby all molecules of the filaments are uniformly relaxed. This is accomplished in our invention by providing a heated zone immediately adjacent to the discharge end of the spinneret through which the emerging filaments pass during the size-reduction draw-down. The zone is of sufficient size so that the time required for the filaments to pass therethrough is such that complete molecular relaxation of the filaments may occur.

The physical apparatus utilized to create the heated zone are by no means critical. A heated fluid (liquid) bath containing a material inert to polystyrene and not a solvent therefor, or a heated gas stream have been found to be adequate. The preferred embodiment, however, is a cylinder-like chimney of metal or other refractory material capable of withstanding elevated temperatures and being provided with electrical or other heating means. The length of the chimney will depend to some extent on the draw rate of the filament which may vary from about 100 feet to about 1400 feet per minute, depending in turn upon the final diameter of the fiber, the rate of extrusion, and the diameter of the orifices in the spinneret. As a general rule, the time required for molecular relaxation from the orifice shear induced orientation is of the order of magnitude of 1 second at temperatures in the range of from 250° C. to 330° C.

After the filaments have been extruded and heat treated to remove the non-uniform orientation, they are permitted to cool under conditions which do not permit re-orientation of a non-uniform nature to occur. In this cold unoriented amorphous state the fibers are quite brittle and difficult to wind on a bobbin. It has been found that this difficulty can be overcome by heating the fibers, prior to the placement on bobbins, at a temperature not high enough to permit orientation. The temperature range of from about 75° C. to about 100° C. is generally suitable for this purpose. It is not necessary to the present process, however, that the fibers be stored on a bobbin prior to being stretch oriented. Even the cold brittle amorphous fibers are sufficiently flexible to permit coiling of the fiber tow in a relatively large diameter drum for storage. Preferably, however, the amorphous fibers are neither wound on a bobbin nor coiled in a drum, but are passed without delay from the heat treating chimney to an orientation bath maintained at a temperature of about 120° C. to about 140° C. After the fibers have been heated in the orientation bath until the temperature of

the fibers is the same as that of the bath, they are passed to a set of godet rolls which impart stretch orientation in an amount of at least 800 percent in the fibers. This high degree of orientation has been found to be required to obtain isotactic polystyrene fibers which have heat stability at approximately 200° C. The rate of stretching found beneficial preferably should have a minimum value of at least 200 ft./min. and a maximum value of about 3000 ft./min.

The process of the present invention is better illustrated by consideration of the following detailed description of a preferred embodiment thereof in conjunction with the drawings, in which:

FIG. 1 is a schematic representation of one method of carrying out the process, and

FIG. 2 is a side elevation partially in section of a spinning head having a relaxing chimney attached thereto.

Referring now to FIG. 1, a conventional extrusion press indicated generally by letter "a" comprising a barrel having rotatably positioned therein an extrusion screw, means for driving said screw (screw and driving means not shown), and a hopper 10 for feeding particulate isotactic polystyrene to the channels of the extrusion screw, is provided with a conventional spinning head 12, preferably operated in conjunction with metering pump (not shown) and a relaxation chimney 14. Pre-pyrolyzed isotactic polystyrene is fed through the extruder hopper 10 to the extruder barrel where the driving action of the screw forces it forward along the barrel to a heated zone 16 maintained at a temperature of about 230° C. to about 250° C. and then to heated zone 18 maintained at a temperature of about 250° C. to about 290° C. The combined shearing action of the screw and the heat transfer occurring in heated zones 16 and 18 flux the polystyrene to a viscous mass which is then delivered at a metered uniform rate to spinning head 12. The spinning head, or more particularly the die portion thereof, is maintained at a temperature of 230° C. to about 330° C. Under the pressure exerted by the metering pump, the molten polystyrene is forced through the die orifices of the spinning head at substantially the same temperature as the die itself. The fine fibers of the polymer issuing from the spinneret are maintained at the die temperature by means of heated chimney 14. The length of the chimney is dependent to some extent upon the amount of thickness reduction to be accomplished by hot drawing and to a larger extent upon the rate of hot drawing which may vary from about 10 ft./min. to about 1400 ft./min. depending primarily upon the linear rate of extrusion of the filaments through the spinneret orifices. The length of the chimney must in all events be long enough to provide a heated zone maintained at the extrusion temperature sufficient to permit any molecular orientation induced in the filaments by the shearing stresses of forming and drawing to relax. After complete molecular relaxation is accomplished, the fibers emerge from the end of the chimney 14 and are collected as a fiber tow. The fiber tow is passed around pulley 20 at a temperature sufficient to prevent the fibers from being too brittle for handling, but at a temperature at which the polymer will not flow or permit orientation. Pulley 20 serves only as a direction changing means for the tow and may be replaced by any conventional equivalent means for accomplishing the same results. From the pulley 20, the tow passes to a pair of rolls 22 through which the force is applied to the fibers in the relaxing chimney to bring about the size reduction by hot drawing. The tow then passes to a constant temperature bath 24, advantageously of glycerine in which the amorphous fiber tow is brought to a temperature of about 125° C. to about 135° C. in preparation for being "cold drawn" to impart uniform, maximum molecular orientation. Stretching of the fiber tow to induce orientation is conveniently accomplished by means of an orientation godet 26, although any means for stretching the tow is within the scope of the

present invention. A stretch ratio of at least 9:1, i.e., 800 percent elongation, is required at 120° C. to 140° C. to form fibers having adequate dimensional stability and strength at room temperature upwards to about 200° C.

One embodiment of a spinning head in combination with a relaxing chimney is shown in detail in FIG. 2. Spinning head is attached to a conduit 28 which conducts the molten polymer stream from the extruder and metering pump into the head 30. The head is bored conventionally in such a way as to change the direction of flow of the molten polymer from horizontal to substantially vertical. The internal bore 31 channels the molten polystyrene to the top of a machined recess into which is fitted a manifold member 32 which serves to maintain uniform pressure and feed across the entire surface area of the multihole die forming member 34. Manifold member 32 and die member 34 are held securely in place in head 30 by means of bolts 36 and 36' ring 38. Constant temperature of the extruder head and die sufficient to maintain the flowing polystyrene in an extrudable condition is provided by electrical band heater 40. Chimney 42 is preferably attached by any suitable means to the spinning head 30 although it is by no means necessary that the chimney be in fact attached so long as the chimney is maintained close to the die orifices. Heater bands 44 maintain the desired temperature in the central portion of the chimney, the temperature being conveniently measured by a thermocouple 46 extending through the side wall of the chimney. The individual fibers as they issue through the forming die and are drawn down within the chimney are caused to converge into a fiber tow at the bottom end of the chimney.

#### EXAMPLE I

Isotactic polystyrene having a melt index of about .01 at 250° C. was pyrolyzed at a temperature of about 395° C. for a period of about 90 seconds to increase the melt index to 10 at 250° C. The pyrolyzed polystyrene in the form of  $\frac{1}{8}$  inch pellets was fed at the rate of about 1 to  $1\frac{1}{2}$  lb./hr. to a 1 inch extruder provided with a spinning head having 50 orifices of 35 mil diameter. The polymer in the extruder barrel was advanced along the barrel by the action of the extrusion screw to a heated zone of the barrel maintained at 160° C. and then to a second zone heated to 260° C., the same temperature at which the spinneret was maintained. As the molten isotactic polystyrene was forced through the spinneret orifices, the resulting filaments were passed through a heated chimney attached to the spinning head and simultaneously hot drawn at the rate of 190 feet per minute. The chimney was maintained at 260° C. and provided a continuous heated passage 18 inches in length. At the draw rate of 190 ft./min. the filaments were reduced in size to about 3 mils in diameter and all shear induced molecular orientation dissipation. As the amorphous filaments emerged from the chimney into air at room temperature they were brought together to form a thread and coiled into a storage drum. The thread was constantly withdrawn from the storage drum at the rate of 20 feet per minute and fed at this rate into a glycerine bath maintained at a temperature of 130° C. to 132° C. The length of thread immersed was 4 feet. From the glycerine bath the thread was picked up by a godet roll travelling at about 190 feet per minute which induced a degree of stretch of about 850 to 900 percent. The final thread had a composite denier of 210, a tensile strength of 2.3 grams per denier, and an extension at break of about 25 percent. Several of these threads obtained as a product of the spinning were plied together to form a heavy knitting yarn. This yarn was textured by allowing a small degree of shrinkage at 135° C. The shrinkage of the individual fibers caused an overall fluffing of the yarn, which when knitted, produced a fabric with good hand and high bulk.

**7**  
**EXAMPLE II**

Fibers of crystallizable isotactic polystyrene having diameters of 20, 10 and 5 mils respectively were formed according to the general method described in Example I and using apparatus similar to that shown in FIG. 1 of the drawings.

|                                       |                                 |      |
|---------------------------------------|---------------------------------|------|
| (a) 20 mil fiber:                     | Melt index of pyrolyzed polymer | 2.5. |
| Extruder conditions—                  |                                 |      |
| First barrel zone                     | 190° C.                         |      |
| Second barrel zone                    | 260° C.                         |      |
| Die (single orifice)                  | 250° C.                         |      |
| Rate of draw down through chimney     | 21 ft./min.                     |      |
| Orientation stretch (rate at 135° C.) | 210 ft./min.                    |      |
| Degree of orientation                 | 900%.                           |      |
| Annealing after orientation           | 10 min. at 135° C.              | 15   |
| (b) 10 mil fiber:                     | Melt index of pyrolyzed polymer | 2.5. |
| Extruder conditions—                  |                                 |      |
| First barrel zone                     | 190° C.                         |      |
| Second barrel zone                    | 260° C.                         |      |
| Die (single orifice)                  | 285° C.                         |      |
| Heated zone (chimney)                 | 285° C.                         |      |
| Rate of draw down through chimney     | 42.5 ft./min.                   |      |
| Orientation stretch (rate at 135° C.) | 425 ft./min.                    |      |
| Degree of orientation                 | 900%.                           |      |
| Annealing after orientation           | 10 min. at 135° C.              |      |
| (c) 5 mil fiber:                      | Melt index of pyrolyzed polymer | 2.5. |
| Extruder conditions—                  |                                 |      |
| First barrel zone                     | 190° C.                         |      |
| Second barrel zone                    | 260° C.                         |      |
| Die (8 hole spinning head)            | 280° C.                         |      |
| Heated zone (chimney)                 | 295° C.                         |      |
| Rate of draw down through chimney     | 30 ft./min.                     |      |
| Orientation stretch (rate at 135° C.) | Constant tension.               |      |
| Degree of orientation                 | 850-900%.                       |      |
| Annealing after orientation           | 10 min. at 135° C.              |      |

The following tables show physical property data of the fibers prepared according to Example II.

*Table I*

| Sample                                | Example II-a  | Example II-b  | Example II-c  |
|---------------------------------------|---------------|---------------|---------------|
| Diameter mils.                        | 20            | 10            | 5             |
| Tensile Strength (lbs./sq. in.)       | 30,000-35,000 | 45,000-50,000 | 40,000-45,000 |
| Extension at break percent.           | 25            | 35            | 30            |
| Tensile Modulus (lbs./sq. in.) (avg.) | 900,000       | 900,000       | 900,000       |
| Modulus (p.s.i.):                     |               |               |               |
| at 25° C.                             | 900,000       |               | 900,000       |
| at 100° C.                            | 400,000       | 400,000       |               |
| at 150° C.                            | 100,000       |               | 100,000       |
| at 175° C.                            | 80,000        | 80,000        |               |
| at 200° C.                            | 75,000        | 75,000        | 75,000        |

The following solvents were found to have no effect on the fibers after 18 hours immersion at 25° C. as determined by tensile strength, tensile modulus, and extension at break:

Xylene  
Turpentine  
Ethylene glycol monoethyl ether  
Isopropyl alcohol  
Mineral spirits

*Table II*

Effect on Tensile Strength, Tensile Modulus, and Extension of Solvent Immersion

|                                        | Before Im-<br>mersion | 18 hrs. in<br>Ethyl<br>Acetate | 18 hrs. in<br>Isobutyl<br>Ketone |
|----------------------------------------|-----------------------|--------------------------------|----------------------------------|
| Tensile Strength (p.s.i.) <sup>1</sup> | 48,000                | 44,000                         | 45,000                           |
| Tensile Modulus (p.s.i.) <sup>1</sup>  | 900,000               | 600,000                        | 700,000                          |
| Extension <sup>1</sup> percent         | 25                    | 30                             | 28                               |

<sup>1</sup> Fiber prepared in Example II-b.

**8**

*Table III*

Shrinkage Characteristics at Elevated Temperatures—  
10 mil Monofil Produced in Example II-b

|    | Temperature: | Percent shrinkage |
|----|--------------|-------------------|
| 10 | 50° C.       | 0.00              |
|    | 100° C.      | 0.25              |
|    | 135° C.      | 0.33              |
|    | 165° C.      | 0.75              |
|    | 200° C.      | 1.50              |

**EXAMPLE III**

Isotactic polystyrene having a melt index of 9.0 after pyrolysis was formed into a 120 denier yarn and tested for tensile strength and extension at break. Using the general method described in Example I and using apparatus similar to that shown in FIG. 1 of the drawings, the following extrusion conditions were employed:

|    | Extruder conditions:                                    |
|----|---------------------------------------------------------|
| 20 | First barrel zone 190° C.                               |
|    | Second barrel zone 250° C.                              |
|    | Die (20 hole-35 ml. spinning) 280° C.                   |
|    | Heated zone (chimney) 283° C.                           |
|    | Rate of draw down through chimney 100 ft./min.          |
| 25 | Orientation stretch (rate at 135° C.) Constant tension. |
|    | Degree of orientation 85%.                              |
|    | Final denier 120.                                       |

30 The following values of tensile strength and extension at break were determined.

| Temperature, ° C. | Tensile Strength (grams/denier) | Extension at Break, percent |
|-------------------|---------------------------------|-----------------------------|
| 25                | 2.7                             | 15                          |
| 45                | 2.3                             | 15                          |
| 70                | 2.0                             | 18                          |
| 90                | 1.8                             | 20                          |
| 110               | 1.4                             | 20                          |
| 150               | 1.4                             | 25                          |
| 175               | 1.0                             | 20                          |
| 200               | 1.0                             | 20                          |

Whereas the foregoing description and examples have been set forth with a certain degree of particularity it is not intended that the scope of the invention be thereby limited.

For instance, the term fiber as used herein is intended to include monofilaments having diameters of up to 20 mils or more, even though an arbitrary distinction is sometimes made in the art between fibers and monofilaments based on diameter size for the sake of convenience.

Since in terms of the present process the critical considerations in producing fibers of less than about 1 mil diameter are substantially the same as in producing monofilaments of greater than about 1 mil diameter, the distinction is not necessary.

What is claimed is:

1. The method for producing isotactic polystyrene textile fibers having uniform molecular orientation which comprises extruding isotactic polystyrene having a melt index of between about 1 and 30 through a die at a temperature between about 230° C. and 330° C. to form a continuous fiber, hot drawing the fiber as it emerges from the die while maintaining the temperature of said fiber substantially at the extrusion temperature until all the molecules of the fiber are completely relaxed, and thereafter cooling the fiber to a temperature of about 120° C. to 140° C. and cold drawing the fiber to impart a degree of stretch of from about 800 to 900 percent whereby a high degree of molecular orientation is induced in said fiber.
2. The method for producing isotactic polystyrene textile fibers having uniform molecular orientation which comprises pyrolyzing isotactic polystyrene at a tempera-

<sup>1</sup> Fiber prepared in Example II-b.

ture between about 325° C. and 425° C. to obtain a polymer having a melt index in the range of about 1 to about 30, extruding the polymer through a die at a temperature between about 230° C. and 330° C. to form a continuous fiber, hot drawing the fiber as it emerges from the die while maintaining the temperature of said fiber substantially at the extrusion temperature until all the fiber molecules are completely relaxed, and thereafter cold drawing the fiber at a temperature in the range of 120° C. to 140° C. to a degree sufficient to impart in said fiber a degree of stretch of about 850 to 900 percent.

3. The method for producing isotactic polystyrene textile fibers having uniform molecular orientation which comprises pyrolyzing isotactic polystyrene at a temperature between about 325° C. and 425° C. to obtain a polymer having a melt index in the range of about 2 to about 20, extruding the polymer through a die at a temperature between about 250° C. and 300° C. to form a continuous fiber, hot drawing the fiber as it emerges from the die through a heated zone maintained at a temperature at least as high as the extrusion temperature and not higher than 330° C. without permitting the temperature of the fiber to fall below the extrusion temperature until all the fiber molecules are completely relaxed, and thereafter cold drawing the fiber at a temperature in the range of 120° C. to 140° C. to stretch said fiber to a degree of about 850 to 900 percent, whereby a high degree of molecular orientation is induced therein.

4. The method according to claim 3 in which the cold drawing is carried out at a temperature in the range of 125° C. to 135° C.

5. The method for producing isotactic polystyrene tex-

tile fibers having uniform molecular orientation which comprises pyrolyzing isotactic polystyrene having a melt index of from about .01 to about 1.0 at a temperature of between about 325° C. and 425° C. to obtain a polymer having a melt index in the range of about 2 to about 20, extruding the polymer through a die at a temperature between about 250° C. and 300° C. to form a continuous fiber, hot drawing the fiber as it emerges from the die through a heated zone maintained at a temperature at least as high as the extrusion temperature and not higher than 330° C. without permitting the temperature of the fiber to fall below the extrusion temperature until all of the fiber molecules are completely relaxed, and thereafter cold drawing the fiber at a rate between 200 ft./min. and 3000 ft./min. and at a temperature of about 135° C. to stretch said fiber a degree of about 850 to 900 per cent whereby a high degree of molecular orientation is induced therein.

References Cited in the file of this patent

UNITED STATES PATENTS

|           |                        |               |
|-----------|------------------------|---------------|
| 2,248,512 | Philip et al. -----    | July 8, 1941  |
| 2,596,128 | Chavannes et al. ----- | May 13, 1952  |
| 2,842,532 | Campbell -----         | July 8, 1958  |
| 2,900,220 | Shaw -----             | Aug. 18, 1959 |
| 2,917,779 | Kurzke et al. -----    | Dec. 22, 1959 |

OTHER REFERENCES

Ser. No. 715,003, Wulff et al. (A.P.C.), published Apr. 30 27, 1943.  
Scientific American, September 1957, page 102 relied upon. (Copy in Scientific Library.)